

# UNITED STATES PATENT OFFICE.

JOHN COULSON, OF WILKINSBURG, PENNSYLVANIA, ASSIGNOR TO WESTINGHOUSE ELECTRIC AND MANUFACTURING COMPANY, A CORPORATION OF PENNSYLVANIA.

## PICKLING PROCESS.

1,374,552.

Specification of Letters Patent. Patented Apr. 12, 1921.

No Drawing.

Application filed October 8, 1917. Serial No. 195,335.

To all whom it may concern:

Be it known that I, JOHN COULSON, a subject of the King of Great Britain, and a resident of Wilkinsburg, in the county of 5 Allegheny and State of Pennsylvania, have invented a new and useful Improvement in Pickling Processes, of which the following is a specification.

My invention relates to the cleansing of 10 metallic objects by electrolytic means, and it has for one of its objects to provide a process of the character indicated, whereby objects of iron, steel and other metals may be effectively cleansed without impairing their 15 strength, resiliency or other physical properties.

Another object of my invention is to provide an electrolytic pickling process by 20 which the surface cleansing of objects of iron or other magnetic material may be combined with an artificial magnetic aging of the material which will tend to prevent further change in the magnetic permeability of such objects.

25 The pickling of iron and steel for the purpose of removing the surface scale has heretofore been performed, either by simple immersion of the objects in acid, usually sulfuric acid, or by making the object to be 30 pickled an electrode of an electrolytic cell having a sulfuric acid electrolyte. It has been found that iron and steel springs and other objects which must necessarily have a high degree of resiliency cannot be satisfactorily pickled by the use of acid alone or 35 as the cathode in an acid electrolyte but become exceedingly brittle on account of the occlusion or adsorption by the metal of the hydrogen evolved in the nascent state upon

40 the surface of the metal in both of these processes. It seems probable that the hydrogen forms an alloy with the metal. It has also been found that the method of pickling in which the object being treated is made the 45 anode of an electrolytic cell is unsatisfactory for the reason that a considerable portion of the material of the anode is removed in the process. For this reason, such iron and steel objects as are injured by an increase in their brittleness or by pitting of 50 their surface are commonly cleansed by sand blasting, instead of by pickling, although the sand blasting treatment is much more expensive and inconvenient.

55 I have discovered that the effect of brit-

tleness of metal treated as a cathode in the pickling process may be overcome by subjecting the treated object to a subsequent treatment as an anode. This removes the hydrogen and restores the elasticity of the material. 60 A small amount of the iron may be dissolved if the treatment during the final step be too long continued, but, in case of springs and other resilient objects, such trifling loss of iron is negligible in view of the substantial 65 gain in strength and permanent magnetic quality effected by my process.

The sulfuric acid electrolyte used in carrying out my process should be concentrated, acid having a specific gravity of about 70 1.20 being suitable for this purpose. The object to be treated is made one electrode and the other electrode, which is preferably of lead, may be the acid-containing tank itself, although this is not essential. The 75 electrodes are preferably connected to the source of electrical energy by a circuit including a reversing switch which is first thrown in such direction that the object being treated is made the cathode and, after 80 the oxid has been removed, is thrown to reverse position to make the treated object the anode. The current density at the anode in the final step of the treatment may suitably be about 60 amperes per square foot. 85 The time required for pickling will vary in accordance with the nature of the material and the thickness of the oxid scale to be removed, and is to be determined as in ordinary pickling methods. Upon finally removing a treated object from the electrolyte, the action of the acid should be stopped 90 by plunging the metal object into water or into a weak alkaline solution.

As stated above, my process not only operates to cleanse the metal but produces a substantial effect upon its magnetic permeability. This appears to result from the liberation of nascent oxygen from the surface of the metal and to a gradually decreasing extent within the pores of the metal, such oxygen combining with the occluded hydrogen which results from the step of removing the oxid, as well as with the occluded oxygen always present in 105 wrought iron and steel.

It is to be understood that the specific materials, proportions and conditions mentioned above are intended to be merely illustrative and not as imposing limitations upon 110

my invention which is defined by the scope of the appended claims.

I claim as my invention:

1. The process that comprises subjecting a ferrous metal, as an electrode of one polarity and subsequently as an electrode of opposite polarity to the action of an electric current in the presence of an electrolyte containing sulfuric acid.
- 10 2. The process that comprises subjecting a ferrous metal as a cathode and subsequently as an anode to the action of an electric current in the presence of an acid electrolyte.
- 15 3. The process of pickling metal that comprises removing the surface scale from the metal and subsequently subjecting the metal, as an anode, to the action of an electric current in the presence of an electrolyte containing an oxygen acid.
- 20 4. The process of pickling metal that comprises electrolytically removing surface oxid from the metal and subsequently subjecting the metal, as an anode, to the action of an electric current in the presence of an acid electrolyte.

5. The process of removing occluded hydrogen from metal that comprises subjecting the metal, as an anode, to the action of an electric current in the presence of an electrolyte containing concentrated sulfuric acid. 30

6. The process of treating steel springs and other metallic objects requiring high resiliency that comprises subjecting the object, as an anode, to the action of an electric current in the presence of an electrolyte, to remove occluded hydrogen from said object. 35

7. The process that comprises immersing a metal object in an electrolyte containing concentrated sulfuric acid and passing an electric current of a density of about 60 amperes per square foot of the surface of the metal object from said object to the electrolyte. 40

8. A magnetic ferrous metal having its magnetic permeability permanently fixed.

In testimony whereof I have hereunto subscribed my name this 27th day of Sept. 1917.

JOHN COULSON.